



US005672562A

**United States Patent**

[19]

Goswami et al.

[11] Patent Number: 5,672,562

[45] Date of Patent: Sep. 30, 1997

## [54] THERMAL RECORDING ELEMENT

[75] Inventors: **Ramanuj Goswami**, Webster; **Robert J. Perry**, Niskayuna; **Paul Anthony Zielinski**, Rochester, all of N.Y.[73] Assignee: **Eastman Kodak Company**, Rochester, N.Y.

[21] Appl. No.: 646,669

[22] Filed: May 8, 1996

[51] Int. Cl.<sup>6</sup> G03C 1/73; G03C 7/02; G01D 15/10

[52] U.S. Cl. 503/227; 430/200; 430/201; 430/334; 430/339; 430/343; 430/964; 346/76 PH

[58] Field of Search 430/200, 201, 430/384, 339, 343, 964; 346/76 PH; 503/227

## [56] References Cited

## U.S. PATENT DOCUMENTS

|           |        |                 |         |
|-----------|--------|-----------------|---------|
| 3,585,038 | 6/1971 | Cescon et al.   | 430/343 |
| 3,734,733 | 5/1973 | Poot et al.     | 430/495 |
| 4,196,002 | 4/1980 | Levinson et al. | 430/617 |
| 4,201,590 | 5/1980 | Levinson et al. | 430/617 |
| 4,894,358 | 1/1990 | Filosa et al.   | 503/201 |
| 5,399,459 | 3/1995 | Simpson et al.  | 430/270 |

*Primary Examiner*—Richard L. Schilling  
*Attorney, Agent, or Firm*—Harold E. Cole

## [57] ABSTRACT

A thermal recording element comprising a support having thereon a dye layer comprising a polymeric binder containing:

(a) a formazan dye that absorbs at from about 400 to about 850 nm, and

(b) a hexaarylbiimidazole which is an oxidative dimer of a 2,4,5-triarylimidazole having one of the following formulas:



7 Claims, No Drawings

## THERMAL RECORDING ELEMENT

This invention relates to a thermal recording element, and more particularly to a thermal recording element containing a formazan dye and a hexaarylbimidazole which is used in a thermal dye-bleaching process to form a monochrome image.

In recent years, thermal transfer systems have been developed to obtain prints from pictures which have been generated electronically from a color video camera. According to one way of obtaining such prints, an electronic picture is first subjected to color separation by color filters. The respective color-separated images are then converted into electrical signals. These signals are then operated on to produce cyan, magenta and yellow electrical signals. These signals are then transmitted to a thermal printer. To obtain the print, a cyan, magenta or yellow dye-donor element is placed face-to-face with a dye-receiving element. The two are then inserted between a thermal printing head and a platen roller. A line-type thermal printing head is used to apply heat from the back of the dye-donor sheet. The thermal printing head has many heating elements and is heated up sequentially in response to one of a cyan, magenta or yellow signal. The process is then repeated for the other two colors. A color hard copy is thus obtained which corresponds to the original picture viewed on a screen. Further details of this process and an apparatus for carrying it out are contained in U.S. Pat. No. 4,621,271, the disclosure of which is hereby incorporated by reference.

U.S. Ser. No. 08/583,395 relates to an antihalation composition and a photothermographic element containing such composition in or on a support. The antihalation composition is described as comprising a formazan dye and a hexaarylbimidazole. There is no disclosure in that application, however, that such a composition would be useful in a thermal recording element for a thermal dye-bleaching process.

U.S. Pat. No. 5,399,459 relates to image formation with thermally bleachable dyes. However, this imaging process involves imagewise dye removal or dye ablation from an element, and not simple bleaching of a dye on a substrate.

U.S. Pat. No. 4,894,358 relates to image formation by bleaching of certain bridged triarylmethane dyes. However, the dye composition employed in the present invention is not disclosed.

It is an object of this invention to provide a thermal recording element comprising a dye layer containing materials which will form a monochrome image upon heating with a thermal head.

This and other objects are achieved in accordance with the invention which comprises a thermal recording element comprising a support having thereon a dye layer comprising a polymeric binder containing:

- (a) a formazan dye that absorbs at from about 400 to about 850 nm, and
- (b) a hexaarylbimidazole (HABI) which is an oxidative dimer of a 2,4,5-triarylimidazole having one of the following formulas:



wherein:

R, R<sup>1</sup> and R<sup>2</sup> each independently represents hydrogen, a substituted or unsubstituted alkyl or alkoxy group of from 1 to about 12 carbon atoms, amino, a substituted or unsubstituted cycloalkyl group having from about 5 to about 7 carbon atoms, or an electron-rich heterocyclic group having from about 5 to about 7 atoms, with the proviso that at least one of R and R<sup>1</sup> is said alkoxy or amino group;

X and X<sup>1</sup> each independently represents oxy or imino;

Z is an alkylene group of 1 or 2 carbon atoms; and

m, n and o each independently represents an integer of 0 to 5.

In the above formulas, R, R<sup>1</sup> and R<sup>2</sup> can represent hydrogen; a substituted or unsubstituted alkyl group of 1 to 12 carbon atoms such as substituted or unsubstituted methyl, ethyl, n-propyl, isopropyl, i-butyl, t-butyl, hexyl, dodecyl, benzyl or neopentyl; a substituted or unsubstituted alkoxy group of 1 to 12 carbon atoms such as substituted or unsubstituted methoxy, ethoxy, 1-propoxy, benzyloxy, ethyleneoxy or dodecyloxy; amino (primary, secondary or tertiary having one or more alkyl groups as defined above); a substituted or unsubstituted cycloalkyl group having 5 to 7 carbon atoms such as substituted or unsubstituted cyclopentyl, cyclohexyl or cycloheptyl; or an electron-rich substituted or unsubstituted heterocyclic group having 5 to 7 atoms (carbon, oxygen, sulfur and nitrogen) in the central ring, such as substituted or unsubstituted furanyl, thiophenyl, pyridyl or pyrrolyl. Other heterocyclic rings would be readily apparent to a skilled artisan.

In a preferred embodiment of the invention, R is an alkoxy group of from 1 to about 8 carbon atoms and o is 1

to 3. In another preferred embodiment,  $R^1$  and  $R^2$  each independently represents a substituted or unsubstituted alkyl or alkoxy group of from 1 to about 4 carbon atoms,  $m$  and  $n$  are each 0 or 1, at least one of  $X$  and  $X^1$  is oxy, and  $Z$  is methylene.

When the compounds have an  $R^1$  or  $R^2$  substituent, it can be located at any position on the respective phenyl rings. Preferably, the one or more  $R^1$  or  $R^2$  groups are in the ortho or para positions of the phenyl rings, in relation to the carbon atoms attached to the imidazole ring. Preferably, when one of  $R^1$  or  $R^2$  is present, it is in the para or 4-position.

In the above formula,  $X$  and  $X^1$  can be the same or different divalent group. Preferably, at least one of them is oxy, and more preferably, each of  $X$  and  $X^1$  is oxy.  $Z$  is alkylene of 1 or 2 carbon atoms, and can be substituted. Preferably,  $Z$  is methylene.

Following are 2,4,5-triarylimidazoles (TAI's) which are used to form the HABI's useful in the invention:



| HABI formed from TAI | R                  | $R^1$   | $R^2$   | $R^3$ |
|----------------------|--------------------|---------|---------|-------|
| R-1                  | $OCH_3$            | H       | H       | H     |
| R-2                  | $OCH_3$            | $OCH_3$ | $OCH_3$ | H     |
| R-3                  | $R-R^1 = -OCH_2O-$ |         | H       | H     |
| R-4                  | $OC_6H_5$          | H       | H       | H     |

The following HABI is an example of the oxidative dimer of the TAI described above:



wherein "Ph" is phenyl.

The TAI radicals dimerize to form the HABI under alkaline oxidative reaction conditions.

Other useful hexaarylbimidazoles are described in U.S. Pat. Nos. 3,383,212, 3,390,994, 3,445,234, 3,533,797, 3,615,481, 3,630,736, 3,666,466 and 3,734,733.

If desired, a combination of hexaarylbimidazoles of the noted structure can be used. These materials can be readily prepared using known preparatory methods described, for example, in U.S. Pat. Nos. 4,196,002 and 4,201,590 to Levinson et al. and by Hayashi, *Bull. Chem. Soc. Japan*, 33, 565 (1960).

Important teachings relating to hexaarylbimidazoles have been published by Aldag, *Photochromism, Molecules and Systems*, Durr and Bouras-Laurent (Eds.), Chapter 18, pages 714-717, Elsevier, 1990. A single triarylimidazole can conceivably give rise to different structural dimers in the dimer linkage made via C—N, C—C or N—N bonds. These individual structural dimers or mixtures thereof can be generated chemically, thermally or photolytically from a common triarylimidazolyl radical. While the dimers specifically described therein are linked via a C—N bond (2-carbon atom of one imidazole ring and nitrogen atom of the other imidazole ring), the present invention is not so limited.

The formazan dyes useful in the present invention absorb at from about 400 to about 850 nm. Preferably, formazan dyes absorbing at from about 500 to about 850 nm are used. Useful formazan dyes are well known in the art, including the Levinson et al. patents cited above, both of which are incorporated herein by reference.

More particularly, useful formazan dyes can be represented by the structure:



wherein:

$R^3$  is a substituted or unsubstituted aromatic group of 6 to 20 atoms in the ring system, such as a carbocyclic or heterocyclic aromatic ring. Such aromatic groups can be carbocyclic or heterocyclic containing one or more nitrogen, oxygen or sulfur atoms. The aromatic group can be substituted with one or more groups as defined below.

$R^4$  can be a substituted or unsubstituted aryl group having from 6 to 14 carbon atoms in the ring system, such as phenyl, tolyl, xylol, naphthyl, anthryl, p-nitrophenyl; or a heterocyclic group having from about 6 to about 14 atoms such as pyridyl, pyrimidyl, oxazolyl, benzothiazolyl, benzimidazolyl.

$R^5$  is a substituted or unsubstituted alkyl group of 1 to 20 carbon atoms, such as substituted or unsubstituted methyl, ethyl, n-propyl, isopropyl, t-butyl, hexyl, decyl, benzyl and other branched or linear hydrocarbons readily apparent to one skilled in the art; a substituted or unsubstituted aryl group of 6 to 14 carbon atoms in the ring, such as phenyl, xylol, tolyl, naphthyl, 4-hydroxyphenyl, p-nitrophenyl, dimethoxyphenyl, anthroquinonyl and other substituted carbocyclic aromatic ring systems readily apparent to one skilled in the art; or a substituted or unsubstituted 5- to 7-membered heterocyclic group having 5 to 7 atoms in the ring nucleus, such as pyridyl, pyrimidyl, oxazolyl, benzothiazolyl, benzimidazolyl, and others readily apparent to one skilled in the art.

Other useful hexaarylbimidazoles are described in U.S. Pat. Nos. 3,383,212, 3,390,994, 3,445,234, 3,533,797, 3,615,481, 3,630,736, 3,666,466 and 3,734,733.

Particularly useful formazan dyes include the following:



F-1

5

**6**  
-continued

F-5



F-2

20



F-3

35



F-4

55



65

F-6

F-7

F-8

10

15

25

30

40

45

50

55

60

-continued



F-9 efficient bleaching by an unknown mechanism. The acid may be added in an amount of from about 0.1 to about 1.0 g/m<sup>2</sup>.

5 As noted above, the thermal recording element of the invention is used to form a dye image. Such a process comprises imagewise healing the thermal recording element, such as by using a thermal head, to form the dye image. This process of forming an image is known as bleaching and forms a monochrome image.

10 Thermal printing heads which can be used to form the dye image by the invention are available commercially. There can be employed, for example, a Fujitsu Thermal Head (FTP-040 MCS001), a TDK Thermal Head F415 HH7-1089 or a Rohm Thermal Head KE 2008-F3. Alternatively, other known sources of energy for thermal dye transfer may be used such as lasers.

15 The following examples are provided to further illustrate 20 the invention.

#### EXAMPLE 1

25 A) A transmissive thermal recording element was prepared by coating a 125  $\mu$ m poly(ethylene terephthalate) support with a subbing layer of poly(acrylonitrile-co-vinylidene 30 chloride-co-acrylic acid) (14:79:7 wt. ratio) (0.08 g/m<sup>2</sup>) and then a mixture of dye and various amounts of HABI R-1 as 35 shown in Tables 1 and 2 below dissolved in 10 g of a 6 wt % solution of poly(vinyl butyral) Butvar 76® (Monsanto Chem. Co.) in acetone with a 125  $\mu$ m doctor blade. The amount of HABI is expressed in terms of molar equivalents of the dye. The coating was allowed to dry for 2 min. at 50° C.

40 F-11 A protective cover sheet was prepared by coating on a 6  $\mu$ m poly(ethylene terephthalate) support a slipping layer of poly(vinyl acetal) (Sekisui Co.) (0.383 g/m<sup>2</sup>), candelilla wax (0.0215 g/m<sup>2</sup>), p-toluenesulfonic acid (0.0003 g/m<sup>2</sup>), and an 45 aminopropyl dimethyl-terminated polydimethylsiloxane, PS513 (Petrarch Systems, Inc.) (0.0108 g/m<sup>2</sup>).

50 B) A reflective thermal recording element was prepared by coating a subbing layer of a mixture of an aminofunctional 45 organo-oxysilane Prosil 221® with a hydrophobic organo-oxysilane, Prosil 2210®, which is an epoxy-terminated organo-oxysilane, was coated onto a support of Oppalyte® polypropylene-laminated paper support with a lightly TiO<sub>2</sub>-pigmented polypropylene skin (Mobil Chemical Co.) at a dry coverage of 0.11 g/m<sup>2</sup>. Prior to coating, the support was subjected to a corona discharge treatment at approximately 450 joules/m<sup>2</sup>.

#### Printing Conditions

55 F-12 The protective cover sheet was placed on top of the thermal recording element, with the slipping layer outermost. This sandwich was then fastened to the top of the motor driven 53 mm diameter rubber roller and a TDK thermal head L-231, thermostated at 24° C. with a head load of 2 kg pressed against the rubber roller. The TDK L-231 thermal print head has 512 independently addressable heaters with a resolution of 5.4 dots/mm and an active printing width of 95 mm, of average heater resistance 512  $\Omega$ . The imaging electronics were activated and the element was drawn between the printing head and roller at 20.6 mm/s. Coincidentally, the resistive elements in the thermal print

A preferred formazan is F-11 wherein R<sup>3</sup> is phenyl, R<sup>4</sup> is benzothiazole, and R<sup>5</sup> is n-propyl.

The preparation of formazan dyes is well known in the art, for example as described by Nineham, *Chem. Reviews*, 55, pp. 355-475 (1955).

Generally, the molar ratio of hexarylbiimidazole to the formazan dye is from about 1:1 to about 5:1. More preferably, this molar ratio is from about 2:1 to about 3:1.

An acid may be added to the dye composition used in the invention such as an organic carboxylic acid or mixture of such acids, each having a pK<sub>a</sub> of from about 3 to about 6. Preferably, the pK<sub>a</sub> is from about 4.5 to about 5.5. Useful acids include, but are not limited to, p-propoxybenzoic acid, o-, p- or m-anisic acid, palmitic acid, 2-chlorobenzoic acid, 1-naphthoic acid, and 4-propylbenzoic acid. A preferred carboxylic acid is o-anisic acid. The acid promotes more

head were pulsed on for 128  $\mu$ s every 130  $\mu$ s. The printing was performed at 12.5 V and 17 ms line time. This translated to an instantaneous power of 0.316 watts/dot and a maximum total printing energy of 5.14 mJ/dot.

The printed image consisted of small squares, each printed at a uniform, but different, energy. A Status A reflective and transmissive density was then obtained on an X-Rite 338 densitometer (X-Rite Corp., Grandville, Mich.) on the recording elements before and after printing. A reading was also made on the blank support for comparison.

TABLE 1

| (Transmissive Support) |      |                  |      |      |                |      |      |     |
|------------------------|------|------------------|------|------|----------------|------|------|-----|
| Dye                    | HABI | Status A Density |      |      |                |      |      |     |
|                        |      | Before           |      |      | After Printing |      |      | (g) |
|                        |      | R                | G    | B    | R              | G    | B    |     |
| F-3<br>(0.010)         | 2    | 0.18             | 0.17 | 0.14 | 0.04           | 0.03 | 0.06 | 25  |
| F-4<br>(0.010)         | 2    | 0.17             | 0.15 | 0.11 | 0.05           | 0.04 | 0.06 |     |
| F-5<br>(0.010)         | 2    | 0.02             | 0.09 | 0.24 | 0.03           | 0.04 | 0.09 |     |
| blank                  |      | 0.02             | 0.02 | 0.02 | 0.02           | 0.02 | 0.02 |     |

TABLE 2

| (Reflective Support) |      |                  |      |      |                |      |      |     |
|----------------------|------|------------------|------|------|----------------|------|------|-----|
| Dye                  | HABI | Status A Density |      |      |                |      |      |     |
|                      |      | Before           |      |      | After Printing |      |      | (g) |
|                      |      | C                | M    | Y    | C              | M    | Y    |     |
| F-3<br>(0.030)       | 4    | 0.46             | 0.45 | 0.48 | 0.42           | 0.34 | 0.48 | 40  |
| F-4<br>(0.030)       | 4    | 1.06             | 1.18 | 0.97 | 0.40           | 0.76 | 0.97 |     |
| F-5<br>(0.030)       | 4    | 1.08             | 1.07 | 0.88 | 0.42           | 0.82 | 0.97 | 45  |
| F-12<br>(0.030)      | 1    | 0.19             | 0.74 | 0.64 | 0.13           | 0.17 | 0.19 |     |
| blank                |      | 0.11             | 0.12 | 0.09 | 0.11           | 0.12 | 0.09 |     |

The above results show that the density decreased (bleached) after printing for the majority of the colors listed for each of the elements. These elements thus functioned as thermal recording elements.

## EXAMPLE 2

Example 1 was repeated except that 0.010 g of dye F-3 was used on a transmissive support. The following results were obtained:

TABLE 3

| 5  | Dye   | HABI | (g) | Molar Equiv. of |      |      | Status A Density |      |      |
|----|-------|------|-----|-----------------|------|------|------------------|------|------|
|    |       |      |     | Before          |      |      | After Printing   |      |      |
|    |       |      |     | R-1             | R    | G    | B                | R    | G    |
|    | F-3   | 1    |     | 0.18            | 0.17 | 0.14 | 0.09             | 0.09 | 0.09 |
| 10 | F-3   | 2    |     | 0.18            | 0.17 | 0.15 | 0.05             | 0.05 | 0.07 |
|    | F-3   | 3    |     | 0.16            | 0.15 | 0.12 | 0.04             | 0.04 | 0.06 |
|    | F-3   | 4    |     | 0.15            | 0.14 | 0.12 | 0.04             | 0.04 | 0.06 |
|    | blank |      |     | 0.02            | 0.02 | 0.02 | 0.02             | 0.02 | 0.02 |

15

The above results show that the density decreased (bleached) after printing, for all of the colors listed for each of the elements. Higher equivalents of HABI provided more efficient bleaching. These elements thus functioned as thermal recording elements.

## EXAMPLE 3

Example 1 was repeated except that a mixture of dyes as shown in Table 4 below was used on a reflective support. In one example, 0.044 g of o-anisic acid was added. The following results were obtained:

TABLE 4

| 35 | Dye F-3/ | HABI | acid  | Molar Equiv. of Status A Density |        |                |      |      |      |
|----|----------|------|-------|----------------------------------|--------|----------------|------|------|------|
|    |          |      |       | (g)                              | Before | After Printing | C    | M    | Y    |
|    | F-5 (g)  | R-1  | (g)   |                                  |        |                |      |      |      |
|    | 0.020/   | 2.8  | 0.044 | 0.65                             | 0.85   | 0.82           | 0.13 | 0.16 | 0.23 |
|    | 0.005    |      |       |                                  |        |                |      |      |      |
|    | 0.020/   | 2.8  | —     | 0.85                             | 0.79   | 0.70           | 0.24 | 0.34 | 0.47 |
|    | 0.005    |      |       |                                  |        |                |      |      |      |
|    | 0.020/   | 4    | —     | 0.85                             | 0.70   | 0.63           | 0.27 | 0.37 | 0.50 |
|    | 0.005    |      |       |                                  |        |                |      |      |      |

The above results show that dye mixtures will also bleach affording the opportunity for making a neutral hue or other desired hues. Also, the addition of an acid enhances bleaching efficiency.

55

## EXAMPLE 4

Example 1 was repeated except that two molar equivalents of various HABI's were used along with 0.020 g of Dye F-3 on a transmissive support. The printing voltage was 13.0 V.

65

Following are HABI comparisons, not within the scope of the invention, used in this experiment:



| HABI formed<br>from TAI | R  | R <sup>1</sup> | R <sup>2</sup> | R <sup>3</sup>   |
|-------------------------|----|----------------|----------------|------------------|
| C-1                     | H  | H              | H              | OCH <sub>3</sub> |
| C-2                     | H  | H              | H              | H                |
| C-3                     | Cl | H              | H              | H                |

**The following results were obtained:**

TABLE 5

| Status A Densities |        |      |      |                |      |      |
|--------------------|--------|------|------|----------------|------|------|
| HABI               | Before |      |      | After Printing |      |      |
|                    | C      | M    | Y    | C              | M    | Y    |
| R-1                | 0.15   | 0.13 | 0.10 | 0.06           | 0.06 | 0.08 |
| R-2                | 0.17   | 0.16 | 0.13 | 0.06           | 0.07 | 0.10 |
| R-3                | 0.13   | 0.12 | 0.10 | 0.06           | 0.06 | 0.09 |
| R-4                | 0.14   | 0.12 | 0.10 | 0.03           | 0.02 | 0.04 |
| C-1                | 0.19   | 0.17 | 0.12 | 0.20           | 0.19 | 0.15 |
| C-2                | 0.19   | 0.17 | 0.13 | 0.19           | 0.17 | 0.14 |
| C-3                | 0.20   | 0.18 | 0.14 | 0.18           | 0.16 | 0.13 |
| Blank              | 0.02   | 0.02 | 0.02 | 0.02           | 0.02 | 0.02 |

The above results show that only the HABI's according to the invention provided good bleaching results as a thermal recording element. The comparison HABI's showed very little bleaching.

### EXAMPLE 5

Example 1 was repeated except that one element contained o-anisic acid, the coatings were on a reflective support and the printing voltage was 13.5 V. The status A yellow densities are reported in Table 6 as the measure of residual yellow D-min of the thermal recording element. The following results were obtained:

TABLE 6

| Dye  | Molar Equiv.<br>of HABI | acid<br>(g) | Status A Yellow Density |                   |                          |
|------|-------------------------|-------------|-------------------------|-------------------|--------------------------|
|      |                         |             | Before<br>Printing      | After<br>Printing | %<br>Density<br>Decrease |
| F-11 | 1.5                     | 0.035       | 1.15                    | 0.21              | 90                       |
| F-3  | 4                       | 0           | 0.51                    | 0.35              | 49                       |

The above results show that both dyes F-11 and F-3 are useful in providing a thermal recording element and F-11 was particularly useful in bleaching yellow density.

The invention has been described in detail with particular reference to preferred embodiments thereof, but it will be

understood that variations and modifications can be effected within the spirit and scope of the invention.

### What is claimed is:

5     1. A process of forming a dye image comprising:  
      imagewise-heating a thermal recording element by using a  
      thermal printing head, said thermal recording element com-  
      prising a support having thereon a dye layer comprising a  
      dye dispersed in a polymeric binder, wherein said dye layer  
10    contains

- (a) a formazan dye that absorbs at from about 400 to about 850 nm. and
  - (b) a hexaarylbiimidazole which is an oxidative dimer of a 2,4,5-triarylimidazole having one of the following formulas:



wherein:

R represents an alkoxy group of from 1 to about 12 carbon atoms:

X and X<sup>1</sup> each independently represents oxy or imino;

Z is an alkylene group of 1 or 2 carbon atoms; and  
 $\alpha$  represents an integer of 1 or 2, with the meaning that

o represents an image of  
when o is 1, then R is in  
is 3, then R is in the pa  
thereby forming said image.

2. The process of claim 1 wherein the molar ratio of said hexaarylbiimidazole to said formazan dye is from about 1:1 to about 5:1.

3. The process of claim 1 wherein R is an alkoxy group of from 1 to about 8 carbon atoms.

4. The process of claim 1 wherein said formazan dye has the structure:



wherein:

R<sup>3</sup> is a substituted or unsubstituted aromatic group of from about 6 to about 20 atoms;

R<sup>4</sup> is a substituted or unsubstituted aryl group having from about 6 to about 14 carbon atoms or a heterocyclic group having from about 6 to about 14 atoms; and

R<sup>5</sup> is a substituted or unsubstituted alkyl group of from 1 to about 20 carbon atoms, a substituted or unsubstituted aryl group of from about 6 to about 14 carbon atoms, or a substituted or unsubstituted heterocyclic ring having from about 5 to about 7 atoms.

5. The process of claim 4 wherein R<sup>3</sup> is phenyl, R<sup>4</sup> is benzothiazole and R<sup>5</sup> is n-propyl.

10. The process of claim 1 wherein said dye layer contains an acid.

6. The process of claim 6 wherein said acid is o-anisic acid.

\* \* \* \* \*